

March 29, 1960

M. COENEN ET AL

2,930,694

OPTICAL SENSITIZATION OF DIRECT POSITIVE EMULSIONS

Filed March 12, 1957

FIG. 1



FIG. 2



FIG. 3



FIG. 4



FIG. 5



INVENTORS:

MAX COENEN, JOHANNES GOETZE, ULRICH GRISAR, OSKAR RIESTER,  
WERNER STRACKE, KARL ZIETAN.

BY Conrad and Hart

their ATTORNEYS

## OPTICAL SENSITIZATION OF DIRECT POSITIVE EMULSIONS

Max Coenen, Krefeld-Uerdingen, Johannes Götz, Köln-Stammheim, Ulrich Grisar, Rheinhausen, Oskar Riester, Leverkusen-Wiesdorf, Werner Stracke, Leverkusen-Bayerwerk, and Karl Zietan, Köln-Stammheim, Germany, assignors to Agfa Aktiengesellschaft, Leverkusen, Germany, a corporation of Germany

Application March 12, 1957, Serial No. 645,544

Claims priority, application Germany March 19, 1956

11 Claims. (Cl. 96—100)

The present invention relates to the sensitizing of direct positive photographic silver salt emulsions. A very large number of dyes have already been proposed for sensitizing silver halide emulsions, many of these dyes originating from the class comprising the polymethine dyes. Nevertheless, this class includes whole groups which have no sensitizing ability or which even have a desensitizing effect. The number of sensitizers which can be used in practice is further restricted by the fact that there is a large number of other requirements concerning the way in which the sensitizer operates when incorporated into silver halide emulsion layers. For example, the clearness of the layers and of the images produced therein must not be reduced and stability on storage, particularly as regards freedom from fogging and intensity of sensitization, must be guaranteed. Furthermore, the gradation in both the fresh and in the aged condition must have the required value and must not change.

For the purposes of color photography, it is only possible to use those sensitizers meeting these requirements which in addition have a particularly high sensitizing action and also a special selectivity. It is even necessary to have a quite specific spectral sensitivity distribution for obtaining the best possible color reproduction. It is obvious that all these requirements can be more or less completely met only by relatively few dyestuffs.

In the modern color photographic processes, the color couplers may be present in the emulsion and these in many cases impair the sensitizing action, whereby the number of dyes which can be used is still further reduced.

The case is particularly complicated when the silver halide emulsions used are those which show the solarization effect, that is to say produce a direct positive silver image when exposed to the object to be reproduced and then developed in a silver halide developing solution. It has actually been found that with direct positive emulsions containing color formers the sensitizers which have formerly been proposed for color photography can be used with only slight success or cannot be used at all.

It has now been found that bis-(1-alkyl-2-phenyl-indole-3)-trimethine cyanines of the general formula



in which:

R is an alkyl radical, such as methyl, ethyl, propyl, butyl  
R' is a hydrogen atom, an alkyl radical, such as methyl, ethyl, propyl, an alkoxy radical such as OCH<sub>3</sub>, OC<sub>2</sub>H<sub>5</sub>.

or a halogen atom, such as chlorine, bromine, iodine, and

R'' is a hydrogen atom or an alkyl such as methyl, ethyl, propyl, butyl, cycloalkyl, such as cyclohexyl, cyclopentyl, thiienyl or R'-C<sub>6</sub>H<sub>4</sub> radical,

5 X is an anion, such as

Cl<sup>-</sup>, Br<sup>-</sup>, I<sup>-</sup>, ClO<sub>4</sub><sup>-</sup>, CH<sub>3</sub>SO<sub>4</sub><sup>-</sup>, C<sub>2</sub>H<sub>5</sub>—SO<sub>4</sub><sup>-</sup>

are particularly suitable for sensitizing direct positive emulsions.

10 These dyes are of a deeper color than the bis-indole-2-cyanines and it has been found that the color of the cyanines of the present invention can moreover be made appreciably deeper by suitable substitution in the 2-position  
15 of the indole ring and by substitution in the trimethine chain.

For example, the dye indicated below as II has an absorption maximum of 595 m $\mu$ , while dye III has an absorption maximum at 615 m $\mu$ .



It is further found that the introduction of the phenyl nuclei has an extremely favorable influence on the sensitizing effect with respect to direct positive emulsions.

35 Fig. 1 shows the sensitization of dye II, and Fig. 2 that of dye III.

It will be seen from these two examples that valuable panchromatic sensitizers for direct positive silver salt emulsions are made available by using bis-(1-alkyl-2-phenyl-indole-3)-trimethine cyanines.

40 It is a surprising fact that the introduction of further substituents, whether these be alkyl or alkoxy groups or halogen atoms, into the benzene ring of the indole does not produce any improvement in the sensitization, as is clear from Fig. 3, which shows the sensitization of dye IV.



45 On the other hand, the introduction of alkyl or alkoxy groups into the phenyl radicals causes a further substantial improvement in the intensity of the sensitization.

50 Fig. 4 shows the sensitization curve of dye V



55 The increase in sensitivity of a direct positive emulsion sensitized with dye V and containing a coupler such as 1-hydroxy-2-naphthoyl - amino-4'-methyl-octadodecylamino-benzene-3'-sulfonic acid for the production of a cyan color image by the process of color forming development, is up to 6° Scheiner as compared with the sensitivity of

an emulsion sensitized with dye III. Dye VI yields practically the same result.



The favorable influence of methyl groups on the 2-phenyl radicals is indicated by Fig. 5 which shows the sensitivity of dye VII.



The alkyl or alkoxy groups or the halogen atoms can however also be introduced into other positions of the 2 phenyl nuclei, for example in the ortho position, as shown for example in dye VIIa.



An even more extensive deepening of the color, and thus a displacement of the sensitization maximum towards longer waves, is caused by the introduction of a thiophene radical into the  $\alpha$ -position of the trimethine chain.

Dye VIII absorbs at  $645 \text{ m}\mu$ , the sensitization maximum is at  $670-680 \text{ m}\mu$ , and dye IX absorbs at  $650 \text{ m}\mu$ .

VIII



IX



The dyes in accordance with the present invention are for example used in such a way that 3-200 mg., preferably at least 60 mg. of one of the said panchromatic sensitizers is used to 1 kg. of a solarized silver halide emulsion. It is, however, possible to use other proportions. The color couplers which are incorporated into said solarized silver salt emulsions are the well known color couplers which are used for the production of color images by the process of color forming develop-

ment. Such couplers are for instance disclosed in U.S. patent specifications 2,179,234, 2,186,849, 2,265,547, 2,276,554, 2,303,928, 2,304,940, 2,322,027, 2,324,832, 2,343,424, 2,357,388, 2,357,395, 2,376,679, 2,376,822, 2,418,748, 2,437,063, 2,449,966, 2,455,169, 2,455,170, 2,453,661.

The dyestuffs illustrated in the above formulae were dissolved in methanol and added to a direct positive emulsion in quantities of 60 mg. per 1 kg. of emulsion.

10 To the sensitized emulsion there were added 10 g. of the sodium salt of sulfonated 1-hydroxy-2-naphthoic acid octadecylamide in the form of a methanolic solution.

When the dyes are dyes which are not substituted in the methine chain, they are produced either by known

15 processes, for example according to W. König, J.pr.Ch. (2), 84, page 216; (2), 87, page 241; Brooker, J. Amer. Chem. Soc. 62 (1940), page 1116, by reacting the corresponding indoles with  $\beta$ -ethoxyacrolein acetal, or, if they are unsymmetrical dyes of the type V, VI, VIII, or IX, 20 by reacting ketones, for example of the formulae



or



35 such as can be obtained for example according to German patent specification No. 614,326, with Grignard compounds to convert them into ethylenes



45 with 3-formyl indoles, which can be obtained from 3-unsubstituted indoles according to Vilsmeier [Berichte der Deutschen Chemischen Gesellschaft, vol. 60 (1927), page 1211], these ethylenes yield the desired dyestuff, for example:



55 in glacial acetic acid solution and in the presence of mineral acids.

60 The following details are given concerning the production of the above dyestuffs:

#### (1) DYESTUFF OF THE FORMULA II

65 *Bis-(1-methyl-2-phenyl-indolyl-3)-trimethine cyanine bromide*

70 2 grams of 1-methyl-2-phenylindole, which can be prepared according to Journ. of the Chem. Soc., London, 1935, page 1210, are heated on a vapor bath until complete dissolution has occurred. 1 gram of  $\beta$ -ethoxy acrolein acetal and 0.8 cc. of hydrobromic acid are added to the hot solution, which is then allowed to cool. After 5 hours, the precipitated dyestuff is filtered off with suction and recrystallized from methanol. The absorption 75 maximum of the dyestuff in alcoholic solution is  $596 \text{ m}\mu$ .

## (2) DYESTUFF OF THE FORMULA III

*Bis-(1-methyl-2-phenylindolyl-3)- $\alpha$ -phenyl trimethine cyanine perchlorate*

(a) 1-methyl-2-phenyl-3-benzoyl-indole:

21 grams of 1-methyl-2-phenylindole,  
20 grams of benzanilide, and  
46 grams of phosphoric oxychloride

are heated in an oil bath to 110° C. for 5 hours, the melt being slowly stirred. Thereupon the reaction mixture is poured into 1 litre of 15% hydrochloric acid, and the mixture is boiled for one hour. After cooling, a smearable mass is deposited at the bottom of the reaction vessel. The dilute acid is decanted, the semi-solid mass ground with water and treated with little methanol after removing the water. The mass solidifies immediately and is filtered off with suction and recrystallized from methanol. The yield is 15 grams, the melting point is 123° C.

(b) Asym.-{1-methyl-2-phenyl-3-benzoylindole} - phenylethylene:

A suspension of 6 grams of 1-methyl-2-phenylindolyl-3 in 30 cc. of benzene is added in small portions to a Grignard solution of 1.5 grams of magnesium, 4 cc. of methyl-iodide and 30 cc. of ether. The mixture is slightly boiled for 2 hours and then mixed with iced water and sulphuric acid. The ether-benzene layer is separated, dried and evaporated. Two grams of a light brown powder are left behind.

(c) Dyestuff formation:

1.5 grams of the ethylene described under (b) and 1.1 grams of 1-methyl-2-phenyl-3-formylindole, described in Journ. of Org. Chemistry, volume 10, page 255 (1945), are dissolved in 15 cc. of hot glacial acetic acid. 0.4 cc. of hydrobromic acid is added and the mixture is allowed to cool. After 4 hours, 0.5 cc. of perchloric acid dissolved in 5 cc. of methanol is added, the mixture is left standing for some hours and the dyestuff perchlorate is filtered off with suction. The filtration residue is alternately washed with methyl and benzene until the lighter soluble red byproduct is separated. Then the dyestuff is recrystallized from methanol. The absorption maximum of the dyestuff in methanolic solution is 615 m $\mu$ .

## (3) DYESTUFF OF THE FORMULA V

*Bis-[1-methyl-2-(p-methoxy-phenyl)-indolyl-3]- $\alpha$ -phenyl trimethine cyanine perchlorate*

(a) 1-methyl - 2 - p-methoxy-phenyl-3-benzoyl-indole:  
72 grams of 1-methyl-2-p-methoxy-phenyl-indole (boiling point 204-208° C. at 2 mm. Hg, prepared from the n-methyl-phenyl-hydrazone of p-methoxy acetophenone by melting with zinc chloride at 180° C.), 60 grams of benzanilide and 135 grams of phosphoric oxychloride are heated to 105° C. for 5 hours. The melt is then decomposed by boiling with 3 litres of 15% hydrochloric acid for 2 hours and immediately poured onto ice. The precipitated mass is filtered off with suction, covered with ethanol and filtered off once more with suction after 12 hours. The residue can be recrystallized from about 1 litre of ethanol. 62 grams of ketone of the melting point 134° C. are obtained.

(b) Asym. - [1 - methyl - 2 - (p-methoxy-phenyl)-indolyl-3]-phenyl-ethylene:

A solution of 30 grams of ketone (a) in 100 cc. benzene is slowly added to a Grignard solution of 6.6 grams of magnesium, 20 cc. of iodomethane and 140 cc. of ether. After the addition is finished, the mixture is heated for 2 hours, then decomposed with ice and sulphuric acid, and the ether-benzene layer is separated. The ether and benzene are substantially evaporated and the ethylene is precipitated with methanol. Melting point at 158° C.

(c) 1-methyl - 2 - p-methoxy-phenyl-3-formyl-indole:

7 grams of N-methyl-formyl-aniline and 7.7 grams of phosphoric oxychloride are left standing at room temperature while stirring for 2 hours. The mixture is then

mixed with 40 grams of o-dichloro-benzene and 11.8 grams of 1-methyl-2-p-methoxy-phenyl-indole are introduced at 50° C. The mixture is left standing for 20 hours and then decomposed with 50 grams of ice and 40 grams of concentrated sodium hydroxide solution while cooling. The dichlorobenzene is distilled off in vacuum and the residue is recrystallized from methanol. Melting point 142° C.

(d) Dyestuff formation:

10 10.2 grams of the asym. ethylene compound (described under (b)) and 8.5 grams of the formyl compound (described under (c)), are dissolved in 100 cc. of hot glacial acetic acid, 3 cc. of hydrobromic acid are added, and the mixture is left standing at room temperature for 5 hours.

15 4 cc. of perchloric acid dissolved in 40 cc. of methanol are added and the dyestuff perchlorate can be filtered off after a further 4 hours. The dyestuff is alternately washed with methanol and benzene several times and then recrystallized from about 3 litres of methanol to which 2 cc. of hydrobromic acid were added. The absorption maximum of the dyestuff in methanolic solution is 625 m $\mu$ .

## (4) DYESTUFF OF THE FORMULA VI

*(1 - methyl - 2 - phenylindolyl - 3)-[1' - methyl-2'-(p-methoxy-phenyl) - indolyl - 3']- $\alpha$ -(p-methoxy - phenyl)-trimethine cyanine perchlorate*

(a) 1-methyl - 2 - phenyl-3-p-methoxy-benzoyl-indole:  
21 grams of 1-methyl-2-phenyl-indole,  
30 24 grams of p-methoxy-benzanilide and  
45 45 grams of phosphoric oxychloride

are treated at 100-105° C. for 5 hours. The reaction mixture is then boiled with 1 litre of 15% hydrochloric acid for 2 hours, poured onto ice and the semi-solid mass is separated by grinding the mass with little ethanol, solidification occurring soon. 20 grams of ketone of the melting point 112° C. are obtained.

(b) Asym.-{1-methyl-2-phenyl-indolyl - 3-(p-methoxy-phenyl)}-ethylene:

40 17 grams of the ketone described in the preceding paragraph dissolved in 60 cc. benzene are added dropwise to a Grignard solution of 3.8 grams of magnesium, 11.4 cc. of iodomethane and 100 cc. of ether. After the reaction is complete, the mixture is kept at boiling temperature for another 2 hours, then decomposed with ice and sulphuric acid, and the ether-benzene mixture is separated off. After drying with sodium sulphate, the solvents are substantially evaporated and the ethylene precipitates with methanol. Yield: 5 grams, melting point 131° C.

(c) Dyestuff formation:

55 1.5 grams of the asym. ethylene obtained as described in the preceding paragraph, and 1.3 grams of 1-methyl-2-(p-methoxy-phenyl)-3-formyl indole, which is obtained as described in Example 3(c), are dissolved in 14 cc. of hot glacial acetic acid. 0.5 cc. of hydrobromic acid is added and the solution is left standing for 4 hours. After adding 0.3 cc. of perchloric acid dissolved in 5 cc. of methanol, the perchlorate of the dyestuff precipitates.

60 The precipitate is filtered off with suction after some hours, alternately washed with methanol and benzene several times, and finally recrystallized from methanol. The absorption maximum in methanolic solution is 625 m $\mu$ .

## (5) DYESTUFF OF THE FORMULA VII

*Bis-[1-methyl-2-(p-methylphenyl)-indolyl-3]-trimethine cyanine bromide*

70 1.5 grams of N-methyl-2-(p-methyl-phenyl)indole are dissolved in 30 cc. of absolute alcohol and heated to the boil. 0.75 cc. of ethoxy acrolein acetal and 0.6 cc. of concentrated hydrobromic acid are added to the hot solution, which is then left standing for 14 hours. During that time crystals precipitate which are filtered off with

suction, washed with benzene and little methanol and then recrystallized from methanol.

(6) DYESTUFF OF THE FORMULA VIII

[1-methyl-2-(p-methoxy-phenyl)-indolyl-3]-[1'-methyl-2'-(p-chlorophenyl)-indolyl-3']- $\alpha$ -( $\alpha$ -thienyl)-trimethine cyanine perchlorate

(a) [1-methyl-2-(p-methoxy-phenyl)-indolyl-3]- $\alpha$ -thienyl-ketone:

6.9 grams of thiophene carbonic acid anilide,  
8 grams of 1-methyl-2-(p-methoxy-phenyl)-indole,  
and  
15 grams of phosphoric oxychloride

are heated to 105° C. for 5 hours. The melt is introduced into hot dilute hydrochloric acid and the mixture is heated to boiling temperature for 2 hours. Thereupon the mixture is poured into ice water, the precipitate formed is filtered off with suction and recrystallized from ethanol. Yield: 7 grams, melting point 140° C.

(b) Asym.-[1-methyl-2-(p-methoxyphenyl)-indolyl-3]- $\alpha$ -thienyl-ethylene:

7 grams of ketone obtained as described in the preceding paragraph dissolved in 15 cc. of benzene are added to a Grignard solution of 1.4 grams of magnesium, 30 cc. of ether and 4 cc. of iodo-methane. After boiling for 2 hours, the mixture is decomposed with ice, acidified with sulphuric acid, the benzene and ether layer is separated, washed and dried. After evaporating the benzene, 5 grams of ethylene of the melting point 115° C. are obtained.

(c) 1-methyl-2-(p-chlorophenyl)-3-formyl-indole:

7 grams of N-methyl-formyl-aniline are stirred with 7.7 grams of phosphoric oxychloride at room temperature for 2 hours. The mixture is diluted with 40 cc. of o-dichlorobenzene and 12 grams of 1-methyl-2-(p-chlorophenyl)-indole are introduced at 5-10° C. The mixture is then left standing for 20 hours, rendered alkaline with concentrated sodium hydroxide solution and ice (the temperature must not rise above 15° C.), the dichlorobenzene is separated, washed neutral, dried and distilled off in vacuum. The residue can be recrystallized from methanol. Yield: 10 grams, melting point 134° C.

(d) Dyestuff formation:

1.7 grams of the ethylene described in 6(b) and 1.35 grams of the aldehyde obtained as described in 6(c) are dissolved in 15 cc. of hot glacial acetic acid. 0.5 cc. of concentrated hydrobromic acid are added to the solution. Formation of the dyestuff starts at once. After 5 hours, 0.5 cc. of perchloric acid dissolved in 50 cc. of methanol is added. After 14 hours, some methanol is added and the precipitated crystals (starting products) are filtered off with suction. Another quantity of 1 cc. of perchloric acid is added to the filtrate, the mixture is then left standing for one day and the resulting precipitate is filtered off again with suction. The residue is washed with much benzene and much alcohol until the effluent no longer shows a red coloration. The residue on the filter is recrystallized from methanol. The pure dyestuff has an absorption maximum in methanolic solution of 645 m $\mu$  and a sensitization maximum of 670 m $\mu$ .

(7) DYESTUFF OF THE FORMULA VIIa

Bis-[1-methyl-2-(o-methyl-phenyl)-indolyl-3]-trimethine cyanine perchlorate

2 grams of 1-methyl-2-(o-methyl-phenyl)-indole,  
25 cc. of absolute alcohol,

1 cc. of ethoxy acrolein acetal, and

0.8 cc. of concentrated hydrochloric acid

are briefly heated on the vapor bath and then left standing for 12 hours. 20 cc. of alcohol and 0.5 cc. of perchloric acid are added, whereupon the dyestuff precipitates immediately. The dyestuff is recrystallized from methanol.

(8) DYESTUFF OF THE FORMULA IX

Bis-[1-methyl-2-(p-methoxy-phenyl)-indolyl-3]- $\alpha$ -( $\alpha$ -thienyl)-trimethine cyanine perchlorate

5 2.5 grams asym.-[1-methyl-2-(p-methoxy-phenyl)-indolyl-3]- $\alpha$ -thienyl ethylene, as described in Example 6(b) and 1.9 grams of 1-methyl-2-p-methoxy-phenyl-3-formyl-indole as described in Example 3(c), are dissolved in 30 cc. of hot glacial acetic acid, 0.7 cc. of hydrobromic acid 10 is added and the mixture is left standing for 6 hours. 1 cc. of perchloric acid dissolved in 10 cc. of methanol is added and the dyestuff formed is filtered off with suction after standing several hours. The dyestuff is washed with benzene and methanol in the usual manner until the effluent no longer shows a red coloration and the dyestuff is then recrystallized from methanol. The absorption maximum of the dyestuff in methanolic solution is 650 m $\mu$ .

15 Suitable direct positive emulsions are disclosed in the patent specification of German Patents No. 606,392, 642,222, 693,917 and 749,864.

We claim:

20 1. A photographic material comprising a direct positive silver halide emulsion layer containing at least one optical sensitizer of the general formula:



35 in which:

R is an alkyl radical,

R' is a member of the group consisting of a hydrogen atom, an alkyl radical, an alkoxy radical, and a halogen atom,

R'' is a member of the group consisting of a hydrogen atom, an alkyl, cycloalkyl, thienyl, and R'-C<sub>6</sub>H<sub>4</sub>-radical,

40 R''' is a member of the class consisting of a hydrogen atom and a methoxy radical, and

X stands for an anion.

2. A photographic material comprising a direct positive silver halide emulsion layer containing a color coupler capable of reacting with the oxidation product of a primary aromatic amino developing agent to form a dye, and also containing at least one optical sensitizer of the general formula:



60 in which:

65 R is an alkyl radical,

R' is a member of the group consisting of a hydrogen atom, an alkyl radical, an alkoxy radical, and a halogen atom,

R'' is a member of the group consisting of a hydrogen atom, an alkyl, cycloalkyl, thienyl, and R'-C<sub>6</sub>H<sub>4</sub>-radical,

R''' is a member of the class consisting of a hydrogen atom and a methoxy radical, and

X stands for an anion.

70 3. A photographic material comprising a direct posi-

9

tive silver halide emulsion layer containing at least one optical sensitizer of the general formula:



4. A photographic material comprising a direct positive silver halide emulsion layer containing at least one optical sensitizer of the general formula:



5. A photographic material comprising a direct positive silver halide emulsion layer containing at least one 20 optical sensitizer of the general formula:



6. A photographic material comprising a direct positive silver halide emulsion layer containing at least one optical sensitizer of the general formula: 30



7. A photographic material comprising a direct positive silver halide emulsion layer containing at least one optical sensitizer of the general formula:



8. A photographic material comprising a direct posi-

10

tive silver halide emulsion layer containing at least one optical sensitizer of the general formula:



9. A photographic material comprising a direct positive silver halide emulsion layer containing at least one optical sensitizer of the general formula:



10. A photographic material comprising a direct positive silver halide emulsion layer containing at least one optical sensitizer of the general formula:



11. A photographic material comprising a direct positive silver halide emulsion layer containing at least one optical sensitizer of the general formula:



**References Cited in the file of this patent**

UNITED STATES PATENTS

- |    |           |                      |               |
|----|-----------|----------------------|---------------|
| 50 | 2,126,078 | Zeh et al. -----     | Aug. 9, 1938  |
|    | 2,640,776 | Spence et al. -----  | June 2, 1953  |
|    | 2,688,545 | Carroll et al. ----- | Sept. 7, 1954 |

#### OTHER REFERENCES

- 55 Mees: "The Theory of the Photographic Process," pages 379 to 391 relied upon (1954); The Macmillan Co., publishers, New York, N.Y. (Copy in Sci. Library.)